

## UNITED STATES PATENT OFFICE.

LOUIS J. REIZENSTEIN, OF PITTSBURGH, PENNSYLVANIA.

## METHOD OF PROCESSING OILS.

No Drawing.

Application filed December 27, 1924. Serial No. 758,444.

This invention relates to castor oil and more particularly to a method of treating castor oil whereby it is rendered miscible in mineral oil at normal temperature.

5 The advantages of obtaining a castor oil (with its remarkable lubricating value under high heats and loads) that is miscible at normal temperatures in mineral oils are many and obvious, and one object of this 10 invention is the provision of a method of processing castor oil whereby it is rendered miscible in mineral oils at normal or ordinary temperatures.

15 The value of a stable mixture of castor oil and a mineral oil in proper proportions to provide a relatively cheap lubricant of high lubricating value is now recognized, especially by aeroplane and automotive engineers and operators as a lubricant for internal 20 combustion engines.

25 Another object of this invention is to produce a mixture of mineral oil and a miscible castor oil. The percentage of castor oil in the mixture will depend upon the duty to 25 which the mixture is to be put and the price at which it is to be sold.

30 I have found that a mixture of mineral oil with a percentage, say from 5% to 40% of castor oil processed in accordance with 30 my invention has remarkable lubricating qualities under high heat and is particularly applicable for use in internal combustion engines.

35 Mixtures of mineral oil of the non-viscous type such as certain of the Russian oils having an extremely low cold test, and castor oil processed in accordance with my invention are valuable as lubricants for use in places where fluidity is required at low 40 temperatures.

45 In processing castor oil, in accordance with my invention, the oil to which a small percentage of inorganic salt has been added is placed in a tank or other suitable open vessel and heated.

50 I have found that a number of inorganic salts may be used, for example, aluminum sulphate, aluminum chloride, aluminum oxide, stannous sulphate, thorium oxide and 50 thorium chloride. Any one of these salts when added in suitable quantity to castor oil will, when the oil is raised to the proper temperature and maintained at such temperature for the required length of time, render 55 the oil miscible in mineral oil. I prefer however, to use aluminum sulphate, since

the processing may be carried out with lower temperatures with this salt than with the others.

All that it is necessary to do is to add 60 about 5 per cent of the salt to the oil and heat the same to a temperature between 150° C. and the decomposition point of the oil. I prefer to heat to about 160° C. Some castor oils require longer heating than others and 65 therefore, it will be advisable to test the oil from time to time in order to find out when it reaches the condition in which it is miscible with mineral oil at normal temperature. When this condition is reached the 70 oil will be poured from the tank or vessel in which it is heated and separated from the salt.

75 By way of example, place 1000 pounds of castor bean oil and 60 pounds of aluminum sulphate in a suitable kettle and raise to a temperature of about 200° C. Hold at this temperature for approximately six to seven hours. Take a small sample of the oil after 80 six or seven hours, allow the same to cool and test for its solubility in cold mineral oil. If it is soluble in cold mineral oil, the reaction is complete. If it is not, it will be necessary to heat for a longer period or until the tests show that it is soluble in cold 85 mineral oil. When the castor bean oil is soluble in mineral oil, the reaction is complete and the mineral salt may be then strained out of the castor oil and the castor oil is then ready for mixing with mineral oil. 90

Under the action of the heat and the inorganic salt the oil gradually takes on its new characteristics. The duration of time of heating, of course, depends upon the temperature to which the oil is raised and the 95 amount of salt used. The higher the temperature the shorter the time of heating and the lower the temperature the longer the time of heating the amount of salt used being the same.

100 Having thus described my invention, what I claim is:—

1. The method of treating castor oil to render it miscible with mineral oil, which consists in heating at atmospheric pressure 105 castor oil in contact with a metallic salt or compound until said oil is miscible with mineral oil at normal temperature then in separating the oil and salt.

2. The method of treating castor oil to 110 render it miscible with mineral oil, which consists in heating castor oil in contact with

aluminum sulphate until said oil is miscible with mineral oil at normal temperature and then in separating the oil and aluminum sulphate.

5 3. The method of treating castor oil to render it miscible with mineral oil, which consists in heating at atmospheric pressure castor oil in contact with aluminum sulphate until said oil is miscible with mineral oil at 10 normal temperature and then in separating the oil and the aluminum sulphate.

4. The method of treating castor oil to render it miscible with mineral oil, which consists in heating at atmospheric pressure 15 raw castor oil to a temperature between 150° C. and the decomposition point of said oil in contact with a metallic salt or com-

pound until said oil is miscible with mineral oil at normal temperature and then in separating the oil and said salt.

20

15. The method of treating castor oil to render it miscible with mineral oil, which consists in heating at atmospheric pressure raw castor oil to a temperature between 150° C. and the decomposition point of said oil in 25 contact with aluminum sulphate until said oil is miscible with mineral oil at normal temperature and then in separating the aluminum sulphate and the oil.

In testimony whereof, I have hereunto 30 subscribed my name this 26th day of December, 1924.

LOUIS J. REIZENSTEIN.